

## UNITED STATES PATENT OFFICE

2,638,410

## BRIGHTENING NICKEL

Walter G. Zelley, New Kensington, Pa., assignor  
to Aluminum Company of America, Pittsburgh,  
Pa., a corporation of Pennsylvania

No Drawing. Application January 16, 1951,  
Serial No. 206,314

5 Claims. (Cl. 41-42)

## 1

This invention relates to solutions and methods for the chemical brightening of nickel. As used herein, the term "nickel" includes pure nickel, commercial nickel containing the usual impurities, nickel base alloys, and nickel plated upon other metals.

According to my invention, nickel surfaces may be readily brightened by simply immersing them for a short time in certain hot aqueous solutions containing phosphoric acid, sulfuric acid and nitric acid.

In the past bright nickel plated surfaces have usually been produced in so-called bright nickel baths, or by buffing the nickel plates produced in so-called dull or semi-bright nickel baths. Bright nickel baths are difficult to maintain in satisfactory condition and do not produce nickel plates having all the desired properties of the other types of baths. On the other hand, buffing is an expensive finishing procedure, and also is not conveniently employed for treating small articles or a variety of different articles. Many efforts have been made to brighten nickel and nickel plated surfaces in simple chemical solutions, but few such treatments have been successful, particularly for the production of surfaces which are both smooth and bright.

An object of this invention is to provide a convenient method for brightening nickel surfaces, particularly nickel plated surfaces. Another object is to provide a simple chemical solution and method for brightening nickel surfaces, thus minimizing or eliminating the need for buffing of such surfaces. These and other objects will be apparent in the following description of the invention.

The solutions that may be employed in accordance with the invention must comprise, as the essential components thereof, on a weight basis referred to the total weight of phosphoric acid, sulfuric acid, nitric acid and water therein, about 45 to 60 per cent phosphoric acid ( $H_3PO_4$ ), about 15 to 25 per cent sulfuric acid ( $H_2SO_4$ ) about 8 to 15 per cent nitric acid ( $HNO_3$ ) and about 10 to 20 per cent water ( $H_2O$ ). The stated water content of the solutions just referred to, and also of those hereinafter referred to, is the entire water content thereof, whether added with the other components or separately. For optimum results such solutions comprising about 50 to 55 per cent phosphoric acid, about 18 to 23 per cent sulfuric acid, about 10 to 13 per cent nitric acid and about 12 to 18 per cent water should be employed.

A solution consisting essentially of the four

5 components specified above, within the limits stated, is very effective for brightening nickel surfaces. However, a solution in which the components specified above constitute but a predominant part of the total is also contemplated. Limited amounts of impurities, dissolved metals or other components may be contained in the solution, for example.

10 The composition of the solution and the temperature at which it is employed are very important. It is only when phosphoric acid, sulfuric acid and nitric acid are mixed in certain proportions, with an appropriate amount of water, that a brightening solution for nickel is produced. Further it is only when such a solution is employed at temperatures above about 65° C. that it is effective for improving the brightness and smoothness of nickel surfaces. To obtain 15 the best results the solution used should be moderately agitated and maintained at a temperature between about 75 and 90° C.

20 The period of immersion will vary with the type of nickel being treated and the temperature of the solution. Generally from about 1 minute to 3 minutes is adequate to effect the removal of about 0.0002 to 0.0003 inches of nickel from the surface being treated, and thus effect good polishing thereof. Shorter periods of time are often sufficient; and longer periods of time may be employed, but do not appear to produce superior 25 results. A single immersion in the solution is, of course, ordinarily sufficient.

30 Surfaces of various types of nickel may be treated in the solution with beneficial results. Surfaces of high brilliancy and smoothness are obtained on nickel plates, for example, thus facilitating the production of smooth plates superimposed thereon.

35 A typical solution for use in accordance with the invention contains the following components:

|           | Per cent by weight |
|-----------|--------------------|
| $H_3PO_4$ | 52                 |
| $H_2SO_4$ | 21                 |
| $HNO_3$   | 12                 |
| $H_2O$    | 15                 |

40 Such a solution may be readily made up from reagent strength acids, as follows:

|                       | Milliliters per liter |
|-----------------------|-----------------------|
| Phosphoric acid (85%) | 600                   |
| Sulfuric acid (96%)   | 200                   |
| Nitric acid (70%)     | 200                   |

45 in which case no added water is required.

50 During use of the solutions described, various

components may be volatilized or decomposed, but the solutions may be readily re-constituted by appropriate additions of components which have reached too low a concentration. Nitric acid additions, for example, must be made from time to time in order to replace amounts which are used up.

It will be understood that brightened nickel surfaces produced in accordance with the invention may be suitably protected by lacquers, employed as a base for chrome plating thereover, or used directly as made.

I claim:

1. A method for chemical brightening of nickel which comprises immersing a nickel article in a solution consisting essentially of about 45 to 60 per cent phosphoric acid, about 15 to 25 per cent sulfuric acid, about 8 to 15 per cent nitric acid and about 10 to 20 per cent water, on a weight basis referred to the total weight of the aforesaid components, the solution being maintained at a temperature above about 65° C.

2. A method for chemical brightening of nickel which comprises immersing a nickel article in a solution consisting essentially of about 50 to 55 per cent phosphoric acid, about 18 to 23 per cent sulfuric acid, about 10 to 13 per cent nitric acid

and about 12 to 18 per cent water, on a weight basis referred to the total weight of the aforesaid components, the solution being maintained at a temperature between about 75 and 90° C.

3. A method according to claim 1 wherein the article is immersed for a period of about 1 to 3 minutes.

4. A method according to claim 2 wherein the article is immersed for a period of about 1 to 3 minutes.

5. A method for chemical brightening of nickel which comprises immersing a nickel article for about 1 to 3 minutes in a solution consisting of about 52 per cent phosphoric acid, about 21 per cent sulfuric acid, about 12 per cent nitric acid and 15 per cent water, on a weight basis, the solution being maintained at a temperature between about 75 and 90° C.

WALTER G. ZELLEY.

References Cited in the file of this patent

UNITED STATES PATENTS

| Number    | Name            | Date          |
|-----------|-----------------|---------------|
| 2,154,455 | Kepfer          | Apr. 18, 1939 |
| 2,337,062 | Page            | Dec. 21, 1943 |
| 2,434,021 | Thompson et al. | Jan. 6, 1948  |